



US007304011B2

(12) **United States Patent**  
**Yaluris et al.**

(10) **Patent No.:** **US 7,304,011 B2**  
(b5) **Date of Patent:** **Dec. 4, 2007**

- (54) **COMPOSITIONS AND PROCESSES FOR REDUCING NO<sub>x</sub> EMISSIONS DURING FLUID CATALYTIC CRACKING**
- (75) Inventors: **George Yaluris**, Columbia, MD (US); **Michael Scott Ziebarth**, Columbia, MD (US); **Xinjin Zhao**, Woodbine, MD (US)
- (73) Assignee: **W.R. Grace & Co. -Conn.**, Columbia, MD (US)
- (\*) Notice: Subject to any disclaimer, the term of this patent is extended or adjusted under 35 U.S.C. 154(b) by 440 days.
- (21) Appl. No.: **10/824,913**
- (22) Filed: **Apr. 15, 2004**
- (65) **Prior Publication Data**  
US 2005/0230285 A1 Oct. 20, 2005
- (51) **Int. Cl.**  
*B01J 29/80* (2006.01)  
*B01J 29/06* (2006.01)
- (52) **U.S. Cl.** ..... **502/65**; 502/66; 502/67; 502/68; 502/73; 502/74; 502/77; 502/78; 502/79
- (58) **Field of Classification Search** ..... 502/65, 502/66, 67, 68, 73, 74, 77, 78, 79  
See application file for complete search history.

(56) **References Cited**

U.S. PATENT DOCUMENTS

- 2,892,801 A 6/1959 Sargent ..... 252/474  
3,036,973 A 5/1962 Nathan et al. ..... 252/474  
3,129,252 A 4/1964 Graham et al. ..... 260/637  
3,184,417 A 5/1965 Hort ..... 252/474  
3,364,136 A 1/1968 Chen et al. ..... 208/120  
3,617,488 A 11/1971 Csicsery ..... 208/59  
3,634,140 A 1/1972 Krusenstierna ..... 136/86 B  
3,894,940 A 7/1975 Scherzer et al. ..... 208/120  
4,199,435 A 4/1980 Chessmore et al. ..... 208/113  
4,290,878 A 9/1981 Blanton, Jr. ..... 208/120  
4,428,827 A 1/1984 Hobbs et al. ..... 208/120  
4,434,147 A 2/1984 Dimpfl et al. ..... 423/325  
4,469,589 A 9/1984 Yoo et al. ..... 208/120  
4,471,070 A 9/1984 Siefert et al. ..... 502/302  
4,472,267 A 9/1984 Yoo et al. ..... 208/120  
4,472,532 A 9/1984 Mooi ..... 502/302  
4,476,245 A 10/1984 Siefert ..... 502/302  
4,495,304 A 1/1985 Yoo et al. ..... 502/66  
4,495,305 A 1/1985 Yoo et al. ..... 502/65  
4,513,091 A 4/1985 Chang et al. ..... 502/71  
4,521,298 A 6/1985 Rosinski et al. ..... 208/120  
4,522,937 A 6/1985 Yoo et al. ..... 502/302  
4,582,815 A 4/1986 Bowes ..... 502/64  
4,642,178 A 2/1987 Yoo et al. ..... 208/113  
4,654,316 A 3/1987 Barri et al. ..... 502/61  
4,708,786 A 11/1987 Occelli ..... 208/120  
4,728,635 A 3/1988 Bhattacharyya ..... 502/304  
4,735,927 A 4/1988 Gerdes ..... 502/64  
4,747,935 A 5/1988 Scherzer ..... 208/120  
4,758,418 A 7/1988 Yoo et al. ..... 423/244

- 4,778,664 A 10/1988 Grinstead ..... 423/235  
4,790,982 A 12/1988 Yoo et al. ..... 423/239  
4,797,266 A 1/1989 Evans ..... 423/328  
4,798,813 A 1/1989 Kato ..... 502/60  
4,810,369 A 3/1989 Scherzer ..... 208/120  
4,812,430 A 3/1989 Child ..... 502/42  
4,812,431 A 3/1989 Child ..... 502/42  
4,818,509 A 4/1989 Dwyer et al. ..... 423/359  
4,826,799 A 5/1989 Cheng et al. ..... 502/301  
4,830,840 A 5/1989 Bhattacharyya ..... 423/239  
4,853,203 A 8/1989 Guth et al. ..... 423/328  
4,855,115 A 8/1989 Imanari et al. ..... 423/239  
4,880,521 A 11/1989 Scherzer ..... 208/120  
4,889,615 A 12/1989 Chin et al. ..... 208/113  
4,895,994 A 1/1990 Cheng et al. ..... 585/270  
4,898,846 A 2/1990 Edwards et al. ..... 502/67  
4,904,627 A 2/1990 Bhattacharyya ..... 502/63  
4,946,581 A 8/1990 van Broekhoven ..... 208/120  
4,952,382 A 8/1990 van Broekhoven ..... 423/244  
4,957,718 A 9/1990 Yoo et al. ..... 423/244  
4,957,892 A 9/1990 Yoo et al. ..... 502/63  
4,963,520 A 10/1990 Yoo et al. ..... 502/64  
4,973,399 A 11/1990 Green et al. ..... 208/120  
4,976,847 A 12/1990 Maxwell et al. ..... 208/120  
4,980,052 A 12/1990 Green et al. ..... 208/120

(Continued)

FOREIGN PATENT DOCUMENTS

WO WO 03/046112 6/2003

*Primary Examiner*—David M Brunsman  
*(74) Attorney, Agent, or Firm*—Charles A. Cross; Beverly J. Artale

(57) **ABSTRACT**

Compositions for reduction of NO<sub>x</sub> generated during a catalytic cracking process, preferably, a fluid catalytic cracking process, are disclosed. The compositions comprise a fluid catalytic cracking catalyst composition, preferably containing a Y-type zeolite, and a particulate NO<sub>x</sub> composition containing particles of a zeolite having a pore size ranging from about 3 to about 7.2 Angstroms and a SiO<sub>2</sub> to Al<sub>2</sub>O<sub>3</sub> molar ratio of less than about 500. Preferably, the NO<sub>x</sub> reduction composition contains NO<sub>x</sub> reduction zeolite particles bound with an inorganic binder. In the alternative, the NO<sub>x</sub> reduction zeolite particles are incorporated into the cracking catalyst as an integral component of the catalyst. Compositions in accordance with the invention are very effective for the reduction of NO<sub>x</sub> emissions released from the regenerator of a fluid catalytic cracking unit operating under FCC process conditions without a substantial change in conversion or yield of cracked products, e.g., gasoline and light olefins. Processes for the use of the compositions are also disclosed.

# US 7,304,011 B2

Page 2

## U.S. PATENT DOCUMENTS

|               |         |                        |           |                  |         |                         |            |
|---------------|---------|------------------------|-----------|------------------|---------|-------------------------|------------|
| 4,985,384 A * | 1/1991  | Gilson .....           | 502/61    | 5,830,346 A      | 11/1998 | Harandi et al. ....     | 208/113    |
| 4,988,432 A   | 1/1991  | Chin .....             | 208/121   | 5,879,645 A      | 3/1999  | Park .....              | 423/213.2  |
| 4,988,654 A   | 1/1991  | Kennedy et al. ....    | 502/84    | 5,908,804 A      | 6/1999  | Menon et al. ....       | 502/38     |
| 5,002,653 A   | 3/1991  | Kennedy et al. ....    | 208/118   | 5,908,806 A      | 6/1999  | Kharas .....            | 502/64     |
| 5,002,654 A   | 3/1991  | Chin .....             | 208/121   | 5,958,818 A      | 9/1999  | Demmel et al. ....      | 502/68     |
| 5,017,538 A   | 5/1991  | Takeshima .....        | 502/64    | 5,985,225 A      | 11/1999 | Ohtsuka .....           | 423/239.2  |
| 5,037,538 A   | 8/1991  | Chin et al. ....       | 208/113   | 5,993,642 A      | 11/1999 | Mohr et al. ....        | 208/46     |
| 5,041,272 A   | 8/1991  | Tamura et al. ....     | 423/239   | 6,017,508 A      | 1/2000  | Millar et al. ....      | 423/700    |
| 5,069,776 A   | 12/1991 | Biswas et al. ....     | 208/120   | 6,033,641 A      | 3/2000  | Hall et al. ....        | 423/239.2  |
| 5,102,530 A   | 4/1992  | Edwards et al. ....    | 208/120   | 6,040,259 A      | 3/2000  | Mohr .....              | 502/67     |
| 5,114,691 A   | 5/1992  | Pinnavaia et al. ....  | 423/244   | 6,090,271 A      | 7/2000  | Carpency .....          | 208/113    |
| 5,114,898 A   | 5/1992  | Pinnavaia et al. ....  | 502/406   | 6,103,208 A      | 8/2000  | Ogawa et al. ....       | 423/213.2  |
| 5,130,012 A   | 7/1992  | Edwards et al. ....    | 208/113   | 6,103,949 A      | 8/2000  | Demmel et al. ....      | 585/722    |
| 5,145,815 A   | 9/1992  | Zarchy .....           | 502/52    | 6,106,697 A      | 8/2000  | Swan et al. ....        | 208/77     |
| 5,171,553 A   | 12/1992 | Li et al. ....         | 423/239   | 6,110,258 A      | 8/2000  | Fraenkel et al. ....    | 95/117     |
| 5,173,278 A   | 12/1992 | Marler .....           | 423/239   | 6,114,265 A      | 9/2000  | Steffens et al. ....    | 502/52     |
| 5,174,980 A   | 12/1992 | Hellring et al. ....   | 423/706   | 6,129,834 A      | 10/2000 | Peters et al. ....      | 208/120.01 |
| 5,190,736 A   | 3/1993  | Hellring et al. ....   | 423/706   | 6,143,167 A      | 11/2000 | Peters et al. ....      | 208/113    |
| 5,206,196 A   | 4/1993  | Nakano et al. ....     | 502/73    | 6,143,681 A      | 11/2000 | Sachtlef et al. ....    | 502/74     |
| 5,208,198 A   | 5/1993  | Nakano et al. ....     | 502/74    | 6,165,933 A      | 12/2000 | Peters et al. ....      | 502/330    |
| 5,236,877 A * | 8/1993  | Gatte .....            | 502/67    | 6,190,538 B1     | 2/2001  | Gosselink et al. ....   | 208/111.01 |
| 5,240,690 A   | 8/1993  | Tang .....             | 423/236   | 6,214,211 B1     | 4/2001  | Itoh .....              | 208/118    |
| 5,260,043 A   | 11/1993 | Li .....               | 423/239.3 | 6,280,607 B1     | 8/2001  | Peters et al. ....      | 208/120.01 |
| 5,260,240 A   | 11/1993 | Guthrie et al. ....    | 502/41    | 6,284,703 B1     | 9/2001  | Ostgard et al. ....     | 502/301    |
| 5,268,089 A   | 12/1993 | Avidan et al. ....     | 208/113   | 6,309,758 B1     | 10/2001 | Schmidt .....           | 428/570    |
| 5,270,024 A   | 12/1993 | Kasahara .....         | 423/213.2 | 6,358,881 B1     | 3/2002  | Peters et al. ....      | 502/304    |
| 5,286,693 A   | 2/1994  | Ino et al. ....        | 502/68    | 6,376,708 B1     | 4/2002  | Morgenstern et al. .... | 562/538    |
| 5,294,332 A   | 3/1994  | Klotz .....            | 208/120   | 6,379,536 B1     | 4/2002  | Peters et al. ....      | 208/120.01 |
| 5,320,822 A   | 6/1994  | Ozin et al. ....       | 423/700   | 6,380,119 B1     | 4/2002  | Grosch et al. ....      | 502/49     |
| 5,364,517 A   | 11/1994 | Dieckmann et al. ....  | 208/121   | 6,395,403 B2     | 5/2002  | Schmidt .....           | 428/570    |
| 5,371,055 A   | 12/1994 | Cormier et al. ....    | 502/65    | 6,413,898 B1     | 7/2002  | Faber et al. ....       | 502/64     |
| 5,372,706 A   | 12/1994 | Buchanan et al. ....   | 208/113   | 6,471,924 B1     | 10/2002 | Feeley .....            | 423/213.5  |
| 5,374,409 A   | 12/1994 | Kasahara .....         | 423/213.2 | 6,479,421 B1     | 11/2002 | Vierheilig .....        | 502/84     |
| 5,374,410 A   | 12/1994 | Grasselli et al. ....  | 423/239   | 6,528,031 B1     | 3/2003  | Park et al. ....        | 423/239.2  |
| 5,382,352 A   | 1/1995  | Hansen et al. ....     | 208/121   | 6,558,533 B2     | 5/2003  | Schmidt et al. ....     | 208/244    |
| 5,413,699 A   | 5/1995  | Chou .....             | 208/113   | 6,660,683 B1     | 12/2003 | Yaluris et al. ....     | 502/241    |
| 5,413,977 A   | 5/1995  | Occelli .....          | 502/68    | 2001/0002426 A1  | 5/2001  | Mohr et al. ....        | 585/407    |
| 5,422,333 A   | 6/1995  | Kano et al. ....       | 502/60    | 2002/0013228 A1  | 1/2002  | Matsumoto et al. ....   | 502/325    |
| 5,427,989 A   | 6/1995  | Kanesaka .....         | 502/66    | 2002/0016259 A1  | 2/2002  | Tsao .....              | 502/324    |
| 5,433,933 A   | 7/1995  | Eshita et al. ....     | 423/213.2 | 2002/0022573 A1  | 2/2002  | Tanada et al. ....      | 502/344    |
| 5,443,803 A   | 8/1995  | Mizuno .....           | 423/213.2 | 2002/0022574 A1  | 2/2002  | Tanada et al. ....      | 502/527.12 |
| 5,472,677 A   | 12/1995 | Farris et al. ....     | 423/239   | 2002/0037808 A1  | 3/2002  | Ostgard et al. ....     | 502/301    |
| 5,503,818 A   | 4/1996  | Nicolaides et al. .... | 423/327.1 | 2002/0038051 A1  | 3/2002  | Ostgard et al. ....     | 562/538    |
| 5,510,306 A   | 4/1996  | Murray .....           | 502/64    | 2002/0049132 A1  | 4/2002  | Jan et al. ....         | 502/60     |
| 5,536,687 A * | 7/1996  | Ward .....             | 502/67    | 2002/0082159 A1  | 6/2002  | Grosch et al. ....      | 502/38     |
| 5,543,125 A   | 8/1996  | Uchida .....           | 423/239.2 | 2002/0082460 A1  | 6/2002  | Verduijn et al. ....    | 585/475    |
| 5,547,648 A   | 8/1996  | Buchanan et al. ....   | 423/210   | 2002/0094314 A1  | 7/2002  | Miyadera et al. ....    | 423/239.1  |
| 5,565,181 A   | 10/1996 | Dieckmann et al. ....  | 423/239.1 | 2002/0094932 A1  | 7/2002  | Faber et al. ....       | 502/74     |
| 5,599,520 A   | 2/1997  | Garces et al. ....     | 423/700   | 2002/0120169 A1  | 8/2002  | Spagnol et al. ....     | 568/316    |
| 5,614,453 A   | 3/1997  | Occelli .....          | 502/66    | 2002/0139112 A1  | 10/2002 | Onodera et al. ....     | 60/286     |
| 5,627,125 A   | 5/1997  | Ebner et al. ....      | 502/331   | 2002/0160905 A1  | 10/2002 | Loyalka et al. ....     | 502/60     |
| 5,695,728 A   | 12/1997 | Miura .....            | 423/239.2 | 2002/0183191 A1  | 12/2002 | Faber et al. ....       | 502/63     |
| 5,705,053 A   | 1/1998  | Buchanan .....         | 208/113   | 2002/0187098 A1  | 12/2002 | Pinnavaia et al. ....   | 423/702    |
| 5,716,514 A   | 2/1998  | Buchanan .....         | 208/113   | 2002/0189973 A1  | 12/2002 | Henry et al. ....       | 208/74     |
| 5,741,468 A   | 4/1998  | Saito .....            | 423/239.1 | 2002/0192155 A1  | 12/2002 | Sterte et al. ....      | 423/700    |
| 5,744,686 A   | 4/1998  | Gajda .....            | 585/823   | 2003/0019794 A1  | 1/2003  | Schmidt et al. ....     | 208/244    |
| 5,785,947 A   | 7/1998  | Zones et al. ....      | 423/705   | 2003/0040425 A1  | 2/2003  | Huang et al. ....       | 502/64     |
| 5,807,528 A   | 9/1998  | Nakona et al. ....     | 423/213.2 | 2003/0073566 A1  | 4/2003  | Marshall et al. ....    | 502/64     |
| 5,827,793 A   | 10/1998 | Hu .....               | 502/41    | 2003/0166453 A1* | 9/2003  | Kuvettu et al. ....     | 502/68     |

\* cited by examiner

FIGURE



## 1

**COMPOSITIONS AND PROCESSES FOR  
REDUCING NO<sub>x</sub> EMISSIONS DURING  
FLUID CATALYTIC CRACKING**

**FIELD OF THE INVENTION**

The present invention relates to NO<sub>x</sub> reduction compositions and the method of use thereof to reduce NO<sub>x</sub> emissions in refinery processes, and specifically in fluid catalytic cracking (FCC) processes. More particularly, the present invention relates to NO<sub>x</sub> reduction compositions and the method of use thereof to reduce the content of NO<sub>x</sub> off gases released from a fluid catalytic cracking unit (FCCU) regenerator during the FCC process without a substantial reduction in hydrocarbon conversion or the yield of valuable cracked products.

**BACKGROUND OF THE INVENTION**

In recent years there has been an increased concern in the United States and elsewhere about air pollution from industrial emissions of noxious oxides of nitrogen, sulfur and carbon. In response to such concerns, government agencies have placed limits on allowable emissions of one or more of these pollutants, and the trend is clearly in the direction of increasingly stringent regulations.

NO<sub>x</sub>, or oxides of nitrogen, in flue gas streams exiting from fluid catalytic cracking (FCC) regenerators is a pervasive problem. Fluid catalytic cracking units (FCCUs) process heavy hydrocarbon feeds containing nitrogen compounds, a portion of which is contained in the coke on the catalyst as it enters the regenerator. Some of this coker-nitrogen is eventually converted into NO<sub>x</sub> emissions, either in the FCC regenerator or in a downstream CO boiler. Thus, all FCCUs processing nitrogen-containing feeds can have a NO<sub>x</sub> emissions problem due to catalyst regeneration.

In the FCC process, catalyst particles (inventory) are continuously circulated between a catalytic cracking zone and a catalyst regeneration zone. During regeneration, coke deposited on the cracking catalyst particles in the cracking zone is removed at elevated temperatures by oxidation with oxygen containing gases such as air. The removal of coke deposits restores the activity of the catalyst particles to the point where they can be reused in the cracking reaction. In general, when coke is burned with a deficiency of oxygen, the regenerator flue gas has a high CO/CO<sub>2</sub> ratio and a low level of NO<sub>x</sub>, but when burned with excess oxygen, the flue gas has a high level of NO<sub>x</sub> and a reduced CO content. Thus, CO and NO<sub>x</sub>, or mixtures of these pollutants are emitted with the flue gas in varying quantities, depending on such factors as unit feed rate, nitrogen content of the feed, regenerator design, mode of operation of the regenerator, and composition of the catalyst inventory.

Various attempts have been made to limit the amount of NO<sub>x</sub> gases emitted from the FCCU by treating the NO<sub>x</sub> gases after their formation, e.g., post-treatment of NO<sub>x</sub> containing gas streams as described in U.S. Pat. Nos. 4,434,147, 4,778,664, 4,735,927, 4,798,813, 4,855,115, 5,413,699, and 5,547,648.

Another approach has been to modify the operation of the regenerator to partial burn and then treat the NO<sub>x</sub> precursors in the flue gas before they are converted to NO<sub>x</sub>, e.g., U.S. Pat. Nos. 5,173,278, 5,240,690, 5,372,706, 5,413,699, 5,705,053, 5,716,514, and 5,830,346.

Yet another approach has been to modify the operation of the regenerator as to reduce NO<sub>x</sub> emissions, e.g., U.S. Pat. No. 5,382,352, or modify the CO combustion promoter

## 2

used, e.g., U.S. Pat. Nos. 4,199,435, 4,812,430, and 4,812,431. Enrichment of air with oxygen in a regenerator operating in partial burn mode has also been suggested, e.g., U.S. Pat. No. 5,908,804.

Additives have also been used in attempts to deal with NO<sub>x</sub> emissions. U.S. Pat. Nos. 6,379,536, 6,280,607, 6,129,834 and 6,143,167 disclose the use of NO<sub>x</sub> removal compositions for reducing NO<sub>x</sub> emissions from the FCCU regenerator. U.S. Patent No. 6,165,933 and 6,358,881 also discloses a NO<sub>x</sub> reduction composition, which promotes CO combustion during the FCC catalyst regeneration process step while simultaneously reducing the level of NO<sub>x</sub> emitted during the regeneration step. NO<sub>x</sub> reduction compositions disclosed by these patents may be used as an additive, which is circulated along with the FCC catalyst inventory or incorporated as an integral part of the FCC catalyst.

U.S. Pat. Nos. 4,973,399 and 4,980,052 disclose reducing emissions of NO<sub>x</sub> from the regenerator of the FCCU by incorporating into the circulating inventory of cracking catalyst separate additive particles containing a copper-loaded zeolite.

Many additive compositions heretofore used to control NO<sub>x</sub> emissions have typically caused a significant decrease in hydrocarbon conversion or the yield of valuable cracked products, e.g., gasoline, light olefins and liquefied petroleum gases (LPGs), while increasing the production of coke. It is a highly desirable characteristic for NO<sub>x</sub> additives added to the FCCU not to affect the cracked product yields or change the overall unit conversion. The operation of the FCCU is typically optimized based on the unit design, feed and catalyst to produce a slate of cracked product and maximizes refinery profitability. This product slate is based on the value model of the specific refinery. For example, during the peak summer driving season many refiners want to maximize gasoline production, while during the winter season refiners may want to maximize heating oil production. In other cases a refinery may find it profitable to produce light olefins products that can be sold in the open market or used in an associated petrochemical plant as feedstocks.

When a NO<sub>x</sub> reduction additive increases coke production, the FCCU may have insufficient air capacity to burn the extra coke and may result in a lower feed throughput in the unit. If the additive increases the production of low value dry gas, the production of more valuable products may decrease. An increase in dry gas may exceed the ability of the unit to handle it, thus forcing a reduction of the amount of feed processed. While an additive that increases light olefins production may be desirable if the refinery values these products and the unit has the equipment necessary to process the extra light hydrocarbons, the additive may reduce profitability if the refinery's goal is to maximize gasoline production. Light olefins are typically made in the FCCU at the expense of gasoline production. Even an additive which increases unit conversion may be undesirable if it affects product yields, causes the unit to reach an equipment limitation, and/or decreases the amount of feed that can be processed.

Consequently, any change to the FCCU that affects the product slate or changes the ability to process feed at the desired rate is detrimental to the refinery profitability. Therefore, there exists a need for NO<sub>x</sub> control compositions which do not significantly affect product yields and overall unit conversion.

## SUMMARY OF THE INVENTION

It has now been discovered that the incorporation of a  $\text{NO}_x$  reduction zeolite component with a catalytically cracking catalyst inventory, in particular a cracking catalyst inventory containing an active Y-type zeolite, being circulated throughout a fluid catalytic cracking unit (FCCU) during a fluid catalytic cracking (FCC) process provides superior  $\text{NO}_x$  control performance without substantially reducing or affecting the hydrocarbon conversion or the yield of cracked petroleum products produced during the FCC process.

In accordance with the present invention, novel  $\text{NO}_x$  reduction compositions are provided. Typically, the compositions comprise a particulate composition containing particles of a  $\text{NO}_x$  reduction zeolite component. In a preferred embodiment of the invention, the  $\text{NO}_x$  reduction zeolite particles are bound with an inorganic binder. The binder preferably comprises silica, alumina or silica alumina. Preferably, the  $\text{NO}_x$  reduction zeolite is exchanged with hydrogen, ammonium, alkali metal and combinations thereof. The preferred alkali metal is sodium, potassium and combinations thereof.

In one aspect of the invention, novel zeolite containing  $\text{NO}_x$  reduction compositions are provided which are added to a circulating inventory of the catalytic cracking catalyst as a separate admixture of particles to reduce  $\text{NO}_x$  emissions released from the FCCU regenerator during the FCC process.

In another aspect of the invention, novel  $\text{NO}_x$  reduction compositions are provided which comprise a  $\text{NO}_x$  reduction zeolite incorporated as an integral component of an FCC catalyst, preferably, containing a Y-type zeolite active cracking component.

In yet another aspect of the invention, novel  $\text{NO}_x$  reduction compositions are provided which compositions reduce  $\text{NO}_x$  emissions from the FCCU regenerator during the FCC process while substantially maintaining hydrocarbon conversion and the yield of cracked petroleum products and minimizing an increase in the production of coke.

It is another aspect of the present invention to provide a process for the reduction of the content of  $\text{NO}_x$  in the off gas of the FCCU regenerator during the FCC process using  $\text{NO}_x$  reduction compositions in accordance with the present invention.

Another aspect of the invention is to provide improved FCC processes for the reduction of the content of  $\text{NO}_x$  in the off gases of the FCCU regenerator without substantially affecting hydrocarbon conversion or the yield of petroleum products produced during the FCC process.

These and other aspects of the present invention are described in further detail below.

## BRIEF DESCRIPTION OF THE DRAWINGS

The FIGURE is a graphic representation of the effectiveness of Additive A, Additive B, Additive C, Additive D and Additive E prepared in EXAMPLES 1, 2, 3, 4 and 5 respectively, to reduce  $\text{NO}_x$  emissions from a DCR regenerator versus time on stream, when the additives are blended with an equilibrium cracking catalyst (having the properties as shown in Table 2) which contained 0.25 weight percent of a platinum promoter, CP-3® (obtained from Grace Davison, Columbia, Md.) and deactivated using the Cyclic Propylene Steaming procedure as described in EXAMPLE 6.

## DETAILED DESCRIPTION OF THE INVENTION

Although several nitrogen oxides are known which are relatively stable at ambient conditions, for purposes of the present invention,  $\text{NO}_x$  will be used herein to represent nitric oxide, nitrogen dioxide (the principal noxious oxides of nitrogen) as well as  $\text{N}_2\text{O}_4$ ,  $\text{N}_2\text{O}_5$  and mixtures thereof.

The present invention encompasses the discovery that the use of certain zeolite containing  $\text{NO}_x$  reduction compositions in combination with a fluid catalytic cracking (FCC) catalyst, preferably a catalyst comprising an active Y-type zeolite, is very effective for the reduction of  $\text{NO}_x$  emissions released from the FCCU regenerator under FCC process conditions without a substantial reduction in hydrocarbon feed conversion or the yield of cracked products. Compositions of the invention typically comprise a particulate composition containing particles of a  $\text{NO}_x$  reduction zeolite component. In a preferred embodiment of the invention, the  $\text{NO}_x$  reduction zeolite particles are bound with an inorganic binder. The novel  $\text{NO}_x$  reduction compositions may be added to the circulating inventory of the catalytic cracking catalyst as a separate particle additive or incorporated as an integral component into the cracking catalyst.

For purposes of the present invention, the phrase "a substantial change in hydrocarbon feed conversion or the yield of cracked products" is defined herein to mean in the alternative (i) less than a 30% relative change, preferably less than a 20% relative change and most preferably less than a 10% relative change in the yield of LCO (light cycle oils), bottoms and gasoline in combination with LPG as compared to the baseline yield of the same products; or (ii) less than a 10% relative change, preferably less than a 6.5% relative change and most preferably less than a 5% relative change in the hydrocarbon feed conversion as compared to the baseline conversion. The conversion is defined as 100% times (1—bottoms yield—LCO yield). When the  $\text{NO}_x$  reduction composition is used as a separate additive, the baseline is the mean conversion or yield of a product in the FCCU, operating with the same feed and under the same reaction and unit conditions, but before the additive of the present invention is added to the catalyst inventory. When the  $\text{NO}_x$  reduction composition is integrated or incorporated into the cracking catalyst particles to provide an integral  $\text{NO}_x$  reduction catalyst system, a significant change in the hydrocarbon conversion or yield of cracked products is determined using a baseline defined as the mean conversion or yield of a product in the same FCCU operating with the same feed, under the same reaction and unit conditions, and with a cracking catalyst inventory comprising the same cracking catalyst composition as that containing the  $\text{NO}_x$  reduction composition, except that the  $\text{NO}_x$  reduction composition is replaced in the cracking catalyst with a matrix component such as kaolin or other filler. The percent changes specified above are derived from statistical analysis of DCR operating data.

Zeolites useful as the  $\text{NO}_x$  reduction zeolite component in the present invention include zeolites having a pore size ranging from about 3 to about 7.2 Angstroms with  $\text{SiO}_2$  to  $\text{Al}_2\text{O}_3$  molar ratio of less than about 500, preferably less than 250, most preferably less than 100. Preferably, the  $\text{NO}_x$  reduction zeolite component is a zeolite selected from the group consisting of ZSM-11, beta, MCM-49, mordenite, MCM-56, Zeolite-L, zeolite Rho, erronite, chabazite, clinoptilolite, MCM-22, MCM-35, MCM-61, Offretite, A, ZSM-12, ZSM-23, ZSM-18, ZSM-22, ZSM-57, ZSM-61, ZK-5, NaJ, Nu-87, Cit-1, SSZ-35, SSZ-48, SSZ-44, SSZ-23,

Dachiardite, Merlinite, Lovdarite, Levyne, Laumontite, Epistilbite, Gmelonite, Gismondine, Cancrinite, Brewsterite, Stilbite, Paulingite, Goosecreekite, Natrolite, omega or mixtures thereof. In the most preferred embodiment of the invention, the NO<sub>x</sub> reduction zeolite component is a zeolite selected from the group consisting of beta, MCM-49, mordenite, MCM-56, Zeolite-L, zeolite Rho, erionite, chabazite, clinoptilolite, MCM-22, Offretite, A, ZSM-12, ZSM-23, omega and mixtures thereof.

In a preferred embodiment of the invention, the NO<sub>x</sub> reduction zeolite is exchanged with a material selected from the group consisting of hydrogen, ammonium, alkali metal and combinations thereof, prior to incorporation into the binder or FCC catalyst. The preferred alkali metal is one selected from the group consisting of sodium, potassium and mixtures thereof. Optionally, the NO<sub>x</sub> reduction zeolite may contain stabilizing amounts, e.g., up to about 25 weight percent, of a stabilizing metal (or metal ion), preferably incorporated into the pores of the zeolite. Suitable stabilizing metals include, but are not limited to, metals selected from the group consisting of Groups 2A, 3B, 4B, 5B, 6B, 7B, 8B, 2B, 3A, 4A, 5A, and the Lanthanide Series of The Periodic Table, Ag and mixtures thereof. Preferably, the stabilizing metals are selected from the group consisting of Groups 3B, 2A, 2B, 3A and the Lanthanide Series of the Periodic Table, and mixtures thereof. Most preferably, the stabilizing metals are selected from the group consisting of lanthanum, aluminum, magnesium, zinc, and mixtures thereof. The metal may be incorporated into the pores of the NO<sub>x</sub> reduction zeolite by any method known in the art, e.g., ion exchange, impregnation or the like. For purposes of this invention, the Periodic Table referenced herein above is the Periodic Table as published by the American Chemical Society.

The amount of NO<sub>x</sub> reduction zeolite used in the catalyst/additive compositions of the invention will vary depending upon several factors, including but not limited to, the mode of combining the NO<sub>x</sub> reduction zeolite with the catalytic cracking catalyst and the type of cracking catalyst used. In one embodiment of the invention, the compositions of the invention are separate catalyst/additive compositions and comprise a particulate composition formed by binding particles of a NO<sub>x</sub> reduction zeolite component with a suitable inorganic binder. Generally, the amount of the NO<sub>x</sub> reduction zeolite component present in the particulate compositions of the invention is at least 10, preferably at least 30, most preferably at least 40 and even more preferably at least 50, weight percent based on the total weight of the composition. Typically, the particulate catalyst/additive composition of the invention contains from about 10 to about 85, preferably from about 30 to about 80, most preferably, from about 40 to about 75, weight percent of the NO<sub>x</sub> reduction zeolite component based on the total weight of the catalyst/additive composition.

Binder materials useful to prepare the particulate compositions of the invention include any inorganic binder which is capable of binding a zeolite powder to form particles having properties suitable for use in the FCCU under FCC process conditions. Typical inorganic binder materials useful to prepare compositions in accordance with the present invention include, but are not limited to, alumina, silica, silica-alumina, aluminum phosphate and the like, and mixtures thereof. Preferably, the binder is selected from the group consisting of alumina, silica, silica-alumina. More preferably, the binder comprises alumina. Even more preferably, the binder comprises an acid or base peptized alumina. Most preferably, the binder comprises an alumina sol,

e.g., aluminum chlorohydrol. Generally, the amount of binder material present in the particular catalyst/additive compositions comprises from about 5 to about 50 weight percent, preferably from about 10 to about 30 weight percent, most preferably from about 15 to about 25 weight percent, of the catalyst/additive composition of the invention.

Additional materials optionally present in the compositions of the present invention include, but are not limited to, 10 fillers (e.g., kaolin clay) or matrix materials (e.g., alumina, silica, silica-alumina, yttria, lanthana, ceria, neodymia, samaria, europia, gadolinia, titania, zirconia, praseodymia and mixtures thereof). When used, the additional materials are used in an amount which does not significantly adversely 15 affect the performance of the compositions to reduce NO<sub>x</sub> emissions released from the FCCU regenerator under FCC conditions, the hydrocarbon feed conversion or the product yield of the cracking catalyst. In general the additional materials will comprise no more than about 70 weight 20 percent of the compositions. It is preferred, however, that the compositions of the invention consist essentially of the NO<sub>x</sub> reduction zeolite and an inorganic binder.

Particulate catalyst/additive compositions of the invention should have a particle size sufficient to permit the composition to be circulated throughout the FCCU simultaneously 25 with the inventory of cracking catalyst during the FCC process. Typically the composition of the invention will have a mean particle size of greater than 45  $\mu\text{m}$ . Preferably, the mean particle size is from about 50 to about 200  $\mu\text{m}$ , 30 most preferably from about 55 to about 150  $\mu\text{m}$ , even more preferred from about 60 to about 120  $\mu\text{m}$ . The compositions of the invention typically have a Davison attrition index (DI) value of less than about 50, preferably less than about 20, most preferably less than about 15.

While the present invention is not limited to any particular process of preparation, typically the particulate NO<sub>x</sub> reduction compositions of the invention are prepared by forming an aqueous slurry containing the NO<sub>x</sub> reduction zeolite, the inorganic binder, and optional matrix materials, in an 35 amount sufficient to provide at least 10.0 weight percent of NO<sub>x</sub> reduction zeolite and at least 5.0 weight percent of binder material in the final catalyst/additive composition and, thereafter, spray drying the aqueous slurry to form particles. The spray-dried particles are optionally dried at a 40 sufficient temperature for a sufficient time to remove volatiles, e.g., at about 90° C. to about 320° C. for about 0.5 to about 24 hours. In a preferred embodiment of the invention, the NO<sub>x</sub> reduction zeolite containing aqueous slurry is milled prior to spray-drying to reduce the mean particle size 45 of materials contained in the slurry to 10  $\mu\text{m}$  or less, preferably 5  $\mu\text{m}$  or less, most preferably 3  $\mu\text{m}$  or less. The aqueous slurry may be milled prior to or after incorporation of the binder and/or matrix materials as desired.

The spray-dried composition may be calcined at a temperature 50 and for a time sufficient to remove volatiles and provide sufficient hardness to the binder for use in the FCCU under FCC process conditions, preferably from about 320° C. to about 900° C. from about 0.5 to about 6 hours.

Optionally, the dried or calcined composition is washed or 55 exchanged with an aqueous solution of ammonia or ammonium salt (e.g., ammonium sulfate, nitrate, carbonate, phosphate and the like), or an inorganic or organic acid (e.g., sulfuric, nitric, phosphoric, hydrochloric, acetic, formic and the like) to reduce the amount of alkaline metals, e.g. sodium or potassium, in the finished product.

Particulate compositions of the invention are circulated in the form of separate particle additives along with the main

cracking catalyst throughout the FCCU. Generally, the catalyst/additive composition is used in an amount of at least 0.1 weight percent of the FCC catalyst inventory. Preferably the amount of the catalyst/additive composition used ranges from about 0.1 to about 75 weight percent, most preferably from about 1 to about 50 weight percent of the FCC catalyst inventory. Separate particle catalyst/additive compositions of the invention may be added to the FCCU in the conventional manner, e.g., with make-up catalyst to the regenerator or by any other convenient method.

In a second embodiment of the invention, the  $\text{NO}_x$  reduction zeolite is integrated or incorporated into the cracking catalyst particles themselves to provide an integral  $\text{NO}_x$  reduction catalyst system. In accordance with this embodiment of the invention, the  $\text{NO}_x$  reduction zeolite may be added to the catalyst at any stage during catalyst manufacturing prior to spray drying the cracking catalyst slurry to obtain the fluid cracking catalyst, regardless of any additional optional or required processing steps needed to finish the cracking catalyst preparation. Without intending to limit the incorporation of the  $\text{NO}_x$  reduction zeolite component, and any of the other optional zeolites, within the cracking catalyst to any specific method of cracking catalyst manufacturing, typically the  $\text{NO}_x$  reduction zeolite component, any additional zeolites, the cracking catalyst zeolite, usually USY or REUSY-type, and any matrix materials are slurried in water. The slurry is milled to reduce the mean particle size of solids in the slurry to less than 10  $\mu\text{m}$ , preferably to less than 5  $\mu\text{m}$ , most preferably less than 3  $\mu\text{m}$ . The milled slurry is combined with a suitable matrix and/or binder material, i.e., clay and a silica sol binder. The matrix/binder catalyst material is mixed and then spray-dried. The spray-dried catalyst is optionally washed using an aqueous solution of ammonium hydroxide, an ammonium salt, an inorganic or organic acid, and water to remove the undesirable salts. The washed catalyst may be exchanged with a water soluble rare-earth salt, e.g., rare-earth chlorides, nitrates and the like.

Alternatively, the  $\text{NO}_x$  reduction zeolite component, optional additional zeolites, the cracking catalyst zeolite, any matrix materials, a rare-earth water soluble salt, clay and alumina sol binder are slurried in water and blended. The slurry is milled and spray-dried. The spray-dried catalyst is calcined at about 250° C. to about 900° C. The spray-dried catalyst may then optionally be washed using an aqueous solution of ammonium hydroxide, an ammonium salt, an inorganic or organic acid, and water to remove the undesirable salts. Optionally, the catalyst may be exchanged with a water-soluble rare-earth salt after it has been washed, by any of the methods known in the art.

When integrated into the FCC catalyst particles, the  $\text{NO}_x$  reduction zeolite component typically represents at least about 0.1 weight percent of the FCC catalyst particle. Preferably, the amount of the  $\text{NO}_x$  reduction zeolite component used ranges from about 0.1 to about 60 weight percent, most preferably from about 1 to about 40 weight percent, of the FCC catalyst particles.

In a preferred embodiment of the invention, the FCC cracking catalyst contains a Y-type zeolite. The  $\text{NO}_x$  reduction zeolite may be added as a separate additive particle to a circulating inventory of the cracking catalyst or incorporated directly into the Y-type zeolite containing cracking catalyst as an integral component of the catalyst. In either case, it is preferred that the  $\text{NO}_x$  reduction zeolite be present in that amount sufficient to provide in the total catalyst inventory a ratio of  $\text{NO}_x$  reduction zeolite to Y-type zeolite of less than 2, preferably less than 1.

It is also within the scope of the invention to include additional zeolite components in the catalyst/additive compositions of the invention. The additional zeolite component may be any zeolite which does not adversely affect the  $\text{NO}_x$  reduction performance or cause a substantial reduction or change in cracked product yields during the FCC process. Preferably, the additional zeolite component is a zeolite selected from the group consisting of ferrierite, ZSM-5, ZSM-35 and mixtures thereof. The additional zeolite component is used in any amount that does not significantly adversely affect the performance of the  $\text{NO}_x$  reduction zeolite compositions to reduce  $\text{NO}_x$  emissions and substantially maintain the product yields of the cracking catalyst relative to the use of the cracking catalyst without the  $\text{NO}_x$  reduction catalyst/additive composition. Typically, the additional zeolite component is used in an amount ranging from about 1 to about 80, preferably from about 10 to about 70, weight percent of the catalyst/additive composition. Where the  $\text{NO}_x$  reduction zeolite is used as an integral component of the catalyst, the additional zeolite component is preferably used in an amount ranging from about 0.1 to about 60, most preferably from about 1 to about 40, weight percent of the catalyst composition.

Somewhat briefly, the FCC process involves the cracking of heavy hydrocarbon feedstocks to lighter products by contact of the feedstock in a cyclic catalyst recirculation cracking process with a circulating fluidizable cracking catalyst inventory consisting of particles having a mean size ranging from about 50 to about 150  $\mu\text{m}$ , preferably from about 60 to about 120  $\mu\text{m}$ . The catalytic cracking of these relatively high molecular weight hydrocarbon feedstocks results in the production of a hydrocarbon product of lower molecular weight. The significant steps in the cyclic FCC process are:

- (i) the feed is catalytically cracked in a catalytic cracking zone, normally a riser cracking zone, operating at catalytic cracking conditions by contacting feed with a source of hot, regenerated cracking catalyst to produce an effluent comprising cracked products and spent catalyst containing coke and strippable hydrocarbons;
- (ii) the effluent is discharged and separated, normally in one or more cyclones, into a vapor phase rich in cracked product and a solids rich phase comprising the spent catalyst;
- (iii) the vapor phase is removed as product and fractionated in the FCC main column and its associated side columns to form gas and liquid cracking products including gasoline;
- (iv) the spent catalyst is stripped, usually with steam, to remove occluded hydrocarbons from the catalyst, after which the stripped catalyst is oxidatively regenerated in a catalyst regeneration zone to produce hot, regenerated catalyst which is then recycled to the cracking zone for cracking further quantities of feed.

Conventional FCC catalysts include, for example, zeolite based catalysts with a faujasite cracking component as described in the seminal review by Venuto and Habib, *Fluid Catalytic Cracking with Zeolite Catalysts*, Marcel Dekker, New York 1979, ISBN 0-8247-6870-1, as well as in numerous other sources such as Sadeghbeigi, *Fluid Catalytic Cracking Handbook*, Gulf Publ. Co. Houston, 1995, ISBN 0-88415-290-1. Preferably, the FCC catalyst is a catalyst comprising a Y-type zeolite active cracking component. In a particularly preferred embodiment of the invention, the FCC catalysts consist of a binder, usually silica, alumina, or silica alumina, a Y-type zeolite active component, one or more matrix aluminas and/or silica aluminas, and fillers such as

kaolin clay. The Y-type zeolite may be present in one or more forms and may have been ultra stabilized and/or treated with stabilizing cations such as any of the rare-earths.

Typical FCC processes are conducted at reaction temperatures of 480° C. to 600° C. with catalyst regeneration temperatures of 600° C. to 800° C. As it is well known in the art, the catalyst regeneration zone may consist of a single or multiple reactor vessels. The compositions of the invention may be used in FCC processing of any typical hydrocarbon feedstock. Suitable feedstocks include petroleum distillates or residuals of crude oils having a boiling point range of about 150° C. to about 900° C., preferably, about 200° C. to about 800° C., which when catalytically cracked provide a gasoline or a other petroleum product. Synthetic feeds having boiling points of about 200° C. to about 800° C., such as oil from coal, tar sands or shale oil, can also be included.

In order to remove coke from the catalyst, oxygen or air is added to the regeneration zone. This is performed by a suitable sparging device in the bottom of the regeneration zone, or if desired, additional oxygen is added to the dilute or dense phase of the regeneration zone.

Catalyst/additive compositions in accordance with the invention dramatically reduce, i.e., by at least 10%, preferably at least 20%, the emissions of NO<sub>x</sub> in the FCCU regenerator effluent during the catalyst regeneration, while substantially maintaining the hydrocarbon feed conversion or the yield of cracked products, e.g., gasoline and light olefins, obtained from the cracking catalyst. In some cases, NO<sub>x</sub> reduction of 90% or greater is readily achievable using the compositions and method of the invention without significantly affecting the cracked products yields or feed conversion. However, as will be understood by one skilled in the catalyst art, the extent of NO<sub>x</sub> reduction will depend on such factors as, for example, the composition and amount of the additive utilized; the design and the manner in which the catalytic cracking unit is operated, including but not limited to oxygen level and distribution of air in the regenerator, catalyst bed depth in the regenerator, stripper operation and regenerator temperature, the properties of the hydrocarbon feedstock cracked, and the presence of other catalytic additives that may affect the chemistry and operation of the regenerator. Thus, since each cracking vessel is different in some or all of these respects, the effectiveness of the process of the invention may be expected to vary from unit to unit. NO<sub>x</sub> reduction compositions of the invention also prevent a significant increase in the production of coke during the FCC process.

It is also within the scope of the invention that NO<sub>x</sub> reduction compositions of the invention may be used alone or in combination with one or more additional NO<sub>x</sub> reduction component to achieve NO<sub>x</sub> reduction more efficiently than the use of either of the compositions alone. Preferably, the additional NO<sub>x</sub> reduction component is a non-zeolitic material, that is, a material that contains no or substantially no (i.e., less than 5 weight percent, preferably less than 1 weight percent) zeolite.

One such class of non-zeolitic materials suitable for use in combination with the NO<sub>x</sub> reduction compositions of the invention include noble metal containing NO<sub>x</sub> reduction compositions such as disclosed and described in U.S. Pat. No. 6,660,683 B1, the entire disclosure of which is herein incorporated by reference. Compositions in this class will typically comprise a particulate mixture of (1) an acidic metal oxide containing substantially no zeolite (preferably containing silica and alumina, most preferably containing at least 1 weight percent alumina); (2) an alkali metal (at least 0.5 weight percent, preferably about 1 to about 15 weight

percent), an alkaline earth metal (at least 0.5 weight percent, preferably about 0.5 to about 50 weight percent) and mixtures thereof; (3) at least 0.1 weight percent of an oxygen storage metal oxide component (preferably ceria); and (4) at least 0.1 ppm of a noble metal component (preferably Pt, Pd, Rh, Ir, Os, Ru, Re and mixtures thereof). Preferred compositions in this class of materials comprise (1) an acidic oxide containing at least 50 weight percent alumina and substantially no zeolite; (2) at least 0.5 weight percent of an alkali metal and/or an alkaline earth metal or mixtures thereof; (3) about 1 to about 25 weight percent of an oxygen storage capable transition metal oxide or a rare-earth (preferably, ceria); and (4) at least 0.1 ppm of a noble metal selected from the group consisting of Pt, Rh, Ir, and a combination thereof, all percentage being based on the total weight of the oxidative catalyst/additive composition.

Another class of non-zeolitic materials suitable for use in combination with the NO<sub>x</sub> reduction compositions of the invention include a low NO<sub>x</sub>, CO combustion promoter as disclosed and described in U.S. Pat. Nos. 6,165,933 and 6,358,881, the entire disclosure of these patents being herein incorporated by reference. Typically, the low NO<sub>x</sub> CO combustion promoter compositions comprise (1) an acidic oxide support; (2) an alkali metal and/or alkaline earth metal or mixtures thereof; (3) a transition metal oxide having oxygen storage capability; and (4) palladium. The acidic oxide support preferably contains silica alumina. Ceria is the preferred oxygen storage oxide. Preferably, the NO<sub>x</sub> reduction composition comprises (1) an acidic metal oxide support containing at least 50 weight percent alumina; (2) about 1-10 parts by weight, measured as metal oxide, of at least one alkali metal, alkaline earth metal or mixtures thereof, (3) at least 1 part by weight of CeO<sub>2</sub>; and (4) about 0.01-5.0 parts by weight of Pd, all of said parts by weight of components (2)-(4) being per 100 parts by weight of said acidic metal oxide support material.

Yet another class of non-zeolitic materials suitable for use in combination with the NO<sub>x</sub> reduction compositions of the invention include NO<sub>x</sub> reduction compositions as disclosed and described in U.S. Pat. Nos. 6,379,536, 6,280,607 B1, 6,143,167 and 6,129,834, the entire disclosure of these patents being herein incorporated by reference. In general, the NO<sub>x</sub> reduction compositions comprise (1) an acidic oxide support; (2) an alkali metal and/or alkaline earth metal or mixtures thereof; (3) a transition metal oxide having oxygen storage capability; and (4) a transition metal selected from Groups IB and IIB of the Periodic Table. Preferably, the acidic oxide support contains at least 50 weight percent alumina and preferably contains silica alumina. Ceria is the preferred oxygen storage oxide. In a preferred embodiment of the invention, the NO<sub>x</sub> reduction compositions comprise (1) an acidic oxide support containing at least 50 weight percent alumina; (2) 1-10 weight percent, measured as the metal oxide, of an alkali metal, an alkaline earth metal or mixtures thereof; (3) at least 1 weight percent CeO<sub>2</sub>; and (4) 0.01-5.0 parts weight percent of a transition metal, measured as metal oxide, of Cu or Ag, all parts by weight of components (2)-(4) being per 100 parts by weight of said acidic oxide support.

Another class of non-zeolitic NO<sub>x</sub> reduction materials suitable for use in combination with the NO<sub>x</sub> reduction compositions of the invention include magnesium-aluminum spinels based additives heretofore being useful for the removal of sulfur oxides from a FCC regenerator. Exemplary patents which disclose and describe this type of materials include U.S. Pat. Nos. 4,963,520, 4,957,892, 4,957,718, 4,790,982, 4,471,070, 4,472,532, 4,476,245,

## 11

4,728,635, 4,830,840, 4,904,627, 4,428,827, 5,371,055, 4,495,304, 4,642,178, 4,469,589, 4,758,418, 4,522,937, 4,472,267 and 4,495,305 the entire disclosure of said patents being herein incorporated by reference. Preferably, compositions in this class comprise at least one metal-containing spinel which includes a first metal and a second metal having a valence higher than the valence of said first metal, at least one component of a third metal other than said first and second metals and at least one component of a fourth metal other than said first, second and third metals, wherein said third metal is selected from the group consisting of Group IB metals, Group IIB metals, Group VIA metals, the rare-earth metals, the Platinum Group metals and mixtures thereof, and said fourth metal is selected from the group consisting of iron, nickel, titanium, chromium, manganese, cobalt, germanium, tin, bismuth, molybdenum, antimony, vanadium and mixtures thereof. Preferably, the metal containing spinel comprises magnesium as said first metal and aluminum as said second metal, and the atomic ratio of magnesium to aluminum in said spinel is at least about 0.17. The third metal in the spinel preferably comprises a metal selected from the group consisting of the Platinum Group metals, the rare-earth metals and mixtures thereof. The third metal component is preferably present in an amount in the range of about 0.001 to about 20 weight percent, calculated as elemental third metal, and said fourth metal component is present in an amount in the range of about 0.001 to about 10 weight percent, calculated as elemental fourth metal.

Other non-zeolitic materials useful in combination with the  $\text{NO}_x$  reduction additives of the invention include, but are not limited to, zinc based catalysts such as disclosed and described in U.S. Pat. No. 5,002,654; antimony based  $\text{NO}_x$  reduction additives such as described and disclosed in U.S. Pat. No. 4,988,432; pervoskite-spinel  $\text{NO}_x$  reduction additives such as described and disclosed in U.S. Pat. Nos. 5,364,517 and 5,565,181; hydrotalcite catalyst and additive compositions such as described and disclosed, for example, in U.S. Pat. Nos. 4,889,615, 4,946,581, 4,952,382, 5,114,691, 5,114,898, 6,479,421 B1 and PCT International Publication No. WO 95/03876; and low  $\text{NO}_x$  promoter additive compositions such as described, for example in U.S. Pat. No. 4,290,878; the entire disclosure of each patent being herein incorporated by reference.

It is also within the scope of the invention to use the  $\text{NO}_x$  reduction compositions of the invention in combination with  $\text{NO}_x$  removal compositions as disclosed and described in PCT International Publication Number WO 03/046112 A1, the entire disclosure of which is herein incorporated by reference. Such  $\text{NO}_x$  removal composition generally comprises (i) an acidic oxide support, (ii) cerium oxide, (iii) a lanthanide oxide other than ceria and (iv) optionally, at least one oxide of a transition metal selected from Groups IB and IIB of the Periodic Table, and mixtures thereof.

When used, the additional non-zeolitic  $\text{NO}_x$  reduction compositions are used in an amount sufficient to provide increased  $\text{NO}_x$  reduction when compared to the use of the catalyst/additive compositions alone. Typically, the additional non-zeolitic compositions are used in an amount up to about 50 weight percent of the FCC catalyst inventory. Preferably, the non-zeolitic composition is used in an amount up to about 30 weight percent, most preferably up to about 10 weight percent of the FCC catalyst inventory. The additional  $\text{NO}_x$  reduction composition may be blended with the FCC catalyst inventory as a separate particle additive. Alternatively, the additional  $\text{NO}_x$  reduction composition may be incorporated into the FCC catalyst as an integral component of the catalyst.

## 12

It is also contemplated within the scope of the present invention that catalyst/additive compositions in accordance with the present invention may be used in combination with other additives conventionally used in the FCC process, e.g.; 5 SOX reduction additives, gasoline-sulfur reduction additives, CO combustion promoters, additives for the production of light olefins, and the like.

The scope of the invention is not in any way intended to be limited by the examples set forth below. The examples 10 include the preparation of catalyst/additives useful in the process of the invention and the evaluation of the invention process to reduce  $\text{NO}_x$  in a catalytic cracking environment. The examples are given as specific illustrations of the 15 claimed invention. It should be understood, however, that the invention is not limited to the specific details set forth in the examples.

All parts and percentages in the examples, as well as the remainder of the specification which refers to solid compositions or concentrations, are by weight unless otherwise 20 specified.

Further, any range of numbers recited in the specification or claims, such as that representing a particular set of properties, units of measure, conditions, physical states or 25 percentages, is intended to literally incorporate expressly herein by reference or otherwise, any number falling within such range, including any subset of numbers within any range so recited.

## EXAMPLES

30

## Example 1

A composition containing 40% MCM-49/40% Clay bound with 20% Silica (Additive A) was prepared as follows. 35 An aqueous slurry containing 25% MCM-49 ( $\text{SiO}_2/\text{Al}_2\text{O}_3=18$ ) was milled in a Drais mill. The milled MCM-49 slurry (4880 g) was combined with 1200 g Natka clay (dry basis) and 6000 g silica sol binder (10% solids). The silica sol binder was prepared from sodium silicate and acid alum. 40 The catalyst slurry was then spray dried in a Bowen spray drier. The resulting spray dried product was washed with ammonium sulfate solution, followed by water to give a catalyst with a  $\text{Na}_2\text{O}$  level of less than 0.1 wt %. The properties of the catalyst are shown in Table 1.

45

## Example 2

A composition containing 40% Beta and 40% clay bound with 20% silica sol (Additive B) was prepared as follows. 50 An aqueous slurry containing 21% Beta ( $\text{SiO}_2/\text{Al}_2\text{O}_3=28$ ) was milled in a Drais mill. The milled Beta slurry (5670 g) was combined with 1200 g Natka clay (dry basis) and 6000 g silica sol binder (10% solids). The silica sol binder was prepared from sodium silicate and acid alum. The catalyst 55 slurry was then spray dried in a Bowen spray drier. The resulting spray dried product was washed with ammonium sulfate solution, followed by water to give a catalyst with a  $\text{Na}_2\text{O}$  level of less than 0.1 wt %. The properties of the catalyst are shown in Table 1.

60

## Example 3

A composition containing 40% Mordenite/40% clay bound with 20% silica sol (Additive C) was prepared as follows. 65 An aqueous slurry containing 21% Mordenite ( $\text{SiO}_2/\text{Al}_2\text{O}_3=19$ ) was milled in a Drais mill. The milled Mordenite slurry (3850 g) was combined with 800 g Natka

13

clay (dry basis) and 4000 g silica sol binder (10% solids). The silica sol binder was prepared from sodium silicate and acid alum. The catalyst slurry was then spray dried in a Bowen spray drier. The resulting spray dried product was washed with ammonium sulfate solution, followed by water to give a catalyst with a  $\text{Na}_2\text{O}$  level of less than 0.1 wt %. The properties of the catalyst are shown in Table 1.

## Example 4

A composition containing 40% Zeolite L/40% clay bound with 20% silica sol (Additive D) was prepared as follows. An aqueous slurry containing 25% Zeolite L ( $\text{SiO}_2/\text{Al}_2\text{O}_3=6$ ) was milled in a Drais mill. The milled Zeolite L slurry (5050 g) was combined with 1200 g Natka clay (dry basis) and 6000 g silica sol binder (10% solids). The silica sol binder was prepared from sodium silicate and acid alum. The catalyst slurry was then spray dried in a Bowen spray drier. The resulting spray dried product was washed with ammonium sulfate solution, followed by water to give a catalyst with a  $\text{Na}_2\text{O}$  level of less than 0.1 wt %. The properties of the catalyst are shown in Table 1.

## Example 5

A composition containing 40% MCM-56/40% clay bound with 20% silica sol (Additive E) was prepared as follows. An aqueous slurry containing 21.8% MCM-56 ( $\text{SiO}_2/\text{Al}_2\text{O}_3=19$ ) was milled in a Drais mill. The milled MCM-56 slurry (5765 g) was combined with 1200 g Natka clay (dry basis) and 6000 g silica sol binder (10% solids). The silica sol binder was prepared from sodium silicate and acid alum. The catalyst slurry was then spray dried in a Bowen spray drier. The resulting spray dried product was washed with ammonium sulfate solution, followed by water to give a catalyst with a  $\text{Na}_2\text{O}$  level of less than 0.1 wt %. The properties of the catalyst are shown in Table 1.

TABLE 1

| Properties of Additives A through E. |                       |            |            |            |            |
|--------------------------------------|-----------------------|------------|------------|------------|------------|
|                                      | Additive A            | Additive B | Additive C | Additive D | Additive E |
| TV @ 1750° F.                        | Wt. %                 | 5.68       | 3.72       | 4.76       | 5.11       |
| $\text{SiO}_2$                       | Wt. %                 | 75.9       | 75.1       | 76.3       | 70.5       |
| $\text{Al}_2\text{O}_3$              | Wt. %                 | 23.0       | 22.8       | 22.4       | 17.0       |
| $\text{RE}_2\text{O}_3$              | Wt. %                 | 0.02       | 0.02       | 0.19       | 0.01       |
| $\text{Na}_2\text{O}$                | Wt. %                 | <0.023     | <0.027     | <0.020     | <0.023     |
| Fe                                   | Wt. %                 | 0.44       | 0.44       | 0.43       | 0.23       |
| $\text{TiO}_2$                       | Wt. %                 | 0.96       | 0.95       | 1.10       | 0.52       |
| $\text{K}_2\text{O}$                 | Wt. %                 |            |            |            | 1.681      |
| SA                                   | $\text{m}^2/\text{g}$ | 244        | 238        | 269        | 258        |
| Zeolite                              | $\text{m}^2/\text{g}$ | 182        | 174        | 224        | 196        |
| Matrix                               | $\text{m}^2/\text{g}$ | 62         | 64         | 45         | 62         |
|                                      |                       |            |            |            | 94         |

## Example 6

The ability of Additives A-E to reduce NO emissions from the FCC unit was evaluated using the Davison Circulating Riser (DCR). The description of the DCR has been published in the following papers: G. W. Young, G. D. Weatherbee, and S. W. Davey, "Simulating Commercial FCCU yields with the Davison Circulating Riser (DCR) pilot plant unit," National Petroleum Refiners Association (NPRA) Paper AM88-52; G. W. Young, "Realistic Assessment of FCC Catalyst Performance in the Laboratory," in Fluid Catalytic Cracking: Science and Technology, J. S. Magee

14

and M. M. Mitchell, Jr. Eds., Studies in Surface Science and Catalysis Volume 76, p. 257, Elsevier Science Publishers B.V., Amsterdam 1993, ISBN 0-444-89037-8. The DCR was started up by charging the unit with approximately 1800 g of equilibrium catalyst having properties as shown in Table 2 below. The properties of the additives tested are summarized in Table 1 above. For the purposes of this test, a commercial FCC feed was used having the properties as shown in Table 3 below.

TABLE 2

| Properties of equilibrium catalyst used in DCR tests. |                       |       |
|-------------------------------------------------------|-----------------------|-------|
| $\text{SiO}_2$                                        | wt. %                 | 50.9  |
| $\text{Al}_2\text{O}_3$                               | wt. %                 | 45.5  |
| $\text{RE}_2\text{O}_3$                               | wt. %                 | 0.37  |
| $\text{Na}_2\text{O}$                                 | wt. %                 | 0.37  |
| Fe                                                    | wt. %                 | 0.6   |
| $\text{TiO}_2$                                        | wt. %                 | 1.2   |
| $\text{MgO}$                                          | wt. %                 | 0.319 |
| Ni                                                    | ppm                   | 681   |
| V                                                     | ppm                   | 1160  |
| SA                                                    | $\text{m}^2/\text{g}$ | 188   |
| Zeolite                                               | $\text{m}^2/\text{g}$ | 128   |
| Matrix                                                | $\text{m}^2/\text{g}$ | 60    |

TABLE 3

| Properties of feed used in DCR tests |        |
|--------------------------------------|--------|
| API Gravity @ 60° F.                 | 23.2   |
| Sulfur, wt. %                        | 0.023  |
| Total Nitrogen, wt. %                | 0.13   |
| Basic Nitrogen, wt. %                | 0.0378 |
| Conradson Carbon, wt. %              | 0.03   |
| Fe, ppm                              | 0.7    |
| Na, ppm                              | 0.7    |
| K Factor                             | 11.4   |

TABLE 3-continued

| Properties of feed used in DCR tests |     |
|--------------------------------------|-----|
| Simulated Distillation, vol. %, ° F. |     |
| 5                                    | 453 |
| 20                                   | 576 |
| 40                                   | 660 |
| 60                                   | 743 |

TABLE 3-continued

| Properties of feed used in DCR tests |             |
|--------------------------------------|-------------|
| 80<br>FBP                            | 838<br>1153 |

The DCR was operated with 1% excess O<sub>2</sub> in the regenerator, and with the regenerator operating at 1300° F. (705° C.). After the unit stabilized the baseline NO emissions data were collected using an on-line Lear-Siegler SO<sub>2</sub>/NO Ana-

Hydrocarbon Processing Catalysts, ACS Symposium Series 634, p. 171 (1996), ISBN 0-8412-3411-6.

5 After the unit stabilized again, the NO emissions data were collected and 210 g of the additive to be tested along with 0.525 g of Pt based CO promoter was added to the DCR. The results are recorded in Table 4 below.

10 As shown in that table and the FIGURE, Additives A through E are effective in reducing NO emissions from the DCR regenerator. The additives are especially effective in decreasing NO emissions without significantly affecting the cracked products yields as shown below in Table 5.

TABLE 4

Reduction of NO emissions from the regenerator of the Davison Circulating Riser (DCR) when using Zeolite based additives. TOS is time on stream from the time of adding Pt CO combustion promoter to the unit.

| Additive         | ID #      | Level (%) | TOS (h) | Gas Flow (l/h) | NO* (ppm) | NO Reduction (%) |
|------------------|-----------|-----------|---------|----------------|-----------|------------------|
| ECAT             |           |           |         | 888            | 32        |                  |
| Pt/CPS @ 1450 F. | 18406-35  | 0.25      | 1       | 889            | 156       |                  |
| Additive A       | 18563-115 | 10        | 4       | 906            | 63        | 60               |
| ECAT             |           |           |         | 886            | 49        |                  |
| Pt/CPS @ 1450 F. | 18406-35  | 0.25      | 1.3     | 884            | 148       |                  |
| Additive B       | 18563-116 | 10        | 4       | 917            | 56        | 62               |
| ECAT             |           |           |         | 864            | 27        |                  |
| Pt/CPS @ 1450 F. | 18406-35  | 0.25      | 1.3     | 877            | 124       |                  |
| Additive C       | 18563-112 | 10        | 4       | 912            | 81        | 35               |
| ECAT             |           |           |         | 887            | 19        |                  |
| Pt/CPS @ 1450 F. | 18406-35  | 0.25      | 1.2     | 877            | 125       |                  |
| Additive D       | 18563-117 | 10        | 4       | 913            | 97        | 22               |
| ECAT             |           |           |         | 878            | 39        |                  |
| Pt/CPS @ 1450 F. | 18406-35  | 0.25      | 1.4     | 872            | 152       |                  |
| Additive E       | 18563-114 | 10        | 4       | 864            | 109       | 28               |

TABLE 5

Activity of the cracking catalyst inventory and product yields during testing of zeolite based additives in the DCR.

| Catalyst Name   | ECAT Average of 6 runs | ECAT w/ 0.25% Pt Prom. 10% Additive A | ECAT w/ 0.25% Pt Prom. 10% Additive B | ECAT w/ 0.25% Pt Prom. 10% Additive C | ECAT w/ 0.25% Pt Prom. 10% Additive D | ECAT w/ 0.25% Pt Prom. 10% Additive E |
|-----------------|------------------------|---------------------------------------|---------------------------------------|---------------------------------------|---------------------------------------|---------------------------------------|
| Conversion wt % | 71.07                  | 69.53                                 | 70.92                                 | 71.09                                 | 71.20                                 | 70.38                                 |
| C/O RATIO       | 8.19                   | 7.87                                  | 8.08                                  | 8.19                                  | 7.85                                  | 8.11                                  |
| H2 Yield wt %   | 0.05                   | 0.05                                  | 0.05                                  | 0.05                                  | 0.05                                  | 0.05                                  |
| C1 + C2's wt %  | 1.61                   | 1.70                                  | 1.79                                  | 1.79                                  | 1.73                                  | 1.63                                  |
| Total C3 wt %   | 5.50                   | 6.11                                  | 6.48                                  | 6.23                                  | 5.99                                  | 5.84                                  |
| C3 = wt %       | 4.74                   | 5.08                                  | 5.36                                  | 5.09                                  | 4.98                                  | 5.01                                  |
| Total C4 wt %   | 10.03                  | 9.92                                  | 10.56                                 | 10.47                                 | 10.35                                 | 10.14                                 |
| iC4 wt %        | 3.55                   | 3.65                                  | 4.02                                  | 3.78                                  | 3.80                                  | 3.61                                  |
| Total C4 = wt % | 5.88                   | 5.59                                  | 5.80                                  | 5.98                                  | 5.80                                  | 5.92                                  |
| iC4 = wt %      | 1.63                   | 1.74                                  | 1.80                                  | 1.79                                  | 1.67                                  | 1.77                                  |
| GASOLINE wt %   | 50.95                  | 48.80                                 | 48.69                                 | 49.49                                 | 49.93                                 | 49.74                                 |
| LCO wt %        | 23.84                  | 25.12                                 | 23.94                                 | 23.64                                 | 23.70                                 | 24.37                                 |
| BOTTOMS wt %    | 5.09                   | 5.35                                  | 5.14                                  | 5.27                                  | 5.10                                  | 5.25                                  |
| Coke wt %       | 2.93                   | 2.95                                  | 3.34                                  | 3.07                                  | 3.16                                  | 2.98                                  |

What is claimed is:

1. A fluid cracking catalyst (FCC) composition, which composition comprises (a) a FCC cracking component suitable for catalyzing the cracking of hydrocarbons under FCC conditions, and (b) a particulate NO<sub>x</sub> reduction catalyst/additive composition having a mean particle size of greater than 45  $\mu$ m and comprising (i) at least 10 weight percent of NO<sub>x</sub> reduction zeolite component selected from the group 60 consisting of ZSM-11, beta, MCM-49, mordenite, MCM-56, Zeolite-L, zeolite Rho, erionite, chabazite, clinoptilolite, MCM-22, MCM-35, MCM-61, Offretite, A, ZSM-12, ZSM-65

lyzer (SM8100A). Subsequently, 100 g of catalyst were injected into the DCR consisting of 4.725 g of a commercial sample of a Pt-based combustion promoter (CP®-3) which had been deactivated for 20 h at 1450° F. (788° C.) without any added Ni or V using the Cyclic Propylene Steaming method (CPS). The description of the CPS method has been published in L. T. Boock, T. F. Petti, and J. A. Rudesill, "Contaminant-Metal Deactivation and Metal-Dehydrogenation Effects During Cyclic Propylene Steaming of Fluid Catalytic Cracking Catalysts," Deactivation and Testing of

17

23, ZSM-18, ZSM-22, ZSM-57, ZSM-61, ZK-5, NaJ, Nu-87, Cit-1, SSZ-35, SSZ-48, SSZ-44, SSZ-23, Dachardite, Merlinite, Lovdarite, Levyne, Laumontite, Epistilbite, Gmelonite, Gismondine, Cancrinite, Brewsterite, Stilbite, Paulingite, Goosecreekite, Natrolite, omega or mixtures thereof, and (ii) about 5 to about 50 weight percent of an inorganic binder selected from the group consisting of alumina, silica, silica alumina, alumina phosphate, and mixtures thereof, wherein component (a) and component (b) are separate particles.

2. The catalyst of claim 1 wherein the FCC cracking component contains a Y-type zeolite.

3. The catalyst of claim 2 wherein the NO<sub>x</sub> reduction catalyst/additive composition is present in an amount sufficient to provide a ratio of NO<sub>x</sub> reduction zeolite component to Y-type zeolite of less than 2.

4. The catalyst of claim 1 wherein the amount of NO<sub>x</sub> reduction zeolite component present is at least 30 weight percent of the NO<sub>x</sub> reduction catalyst/additive composition.

5. The catalyst of claim 4 wherein the amount of NO<sub>x</sub> reduction zeolite component present is at least 40 weight percent of the NO<sub>x</sub> reduction catalyst/additive composition.

6. The catalyst of claim 5 wherein the amount of NO<sub>x</sub> reduction zeolite component present at least 50 weight percent of the NO<sub>x</sub> reduction catalyst/additive composition.

7. The catalyst of claim 1 wherein the amount of NO<sub>x</sub> reduction zeolite component present ranges from about 10 to about 85 weight percent of the NO<sub>x</sub> reduction catalyst/additive composition.

8. The catalyst of claim 7 wherein the amount of NO<sub>x</sub> reduction zeolite component present ranges from about 30 to about 80 weight percent of the NO<sub>x</sub> reduction catalyst/additive composition.

9. The catalyst of claim 8 wherein the amount of NO<sub>x</sub> reduction zeolite component present ranges from about 40 to about 75 weight percent of the NO<sub>x</sub> reduction catalyst/additive composition.

10. The catalyst of claim 1 wherein the NO<sub>x</sub> reduction zeolite component is exchanged with a cation selected from the group consisting of hydrogen, ammonium, alkali metal and combinations thereof.

11. The catalyst of claim 1 wherein the NO<sub>x</sub> reduction zeolite component further comprises at least one stabilizing metal.

12. The catalyst of claim 11 wherein the stabilizing metal is a metal selected from the group consisting of Groups 2A, 3B, 4B, 5B, 6B, 7B, 8B, 2B, 3A, 4A, 5A and the Lanthanide Series of the Periodic Table, Ag and mixtures thereof.

13. The catalyst of claim 12 wherein the stabilizing metal is selected from the group consisting of Groups 3B, 2A, 2B, 3A and the Lanthanide Series of the Periodic Table, and mixtures thereof.

14. The catalyst of claim 13 wherein the stabilizing metal is selected from the group consisting of lanthanum, aluminum, magnesium and zinc, and mixtures thereof.

15. The catalyst of claim 11 wherein the stabilizing metal is incorporated into the pores of the NO<sub>x</sub> reduction zeolite component.

16. The catalyst of claim 1 wherein the inorganic binder in the particulate NO<sub>x</sub> reduction catalyst/additive composition is selected from the group consisting of silica, alumina, silica alumina and mixtures thereof.

17. The catalyst of claim 16 wherein the inorganic binder is alumina.

18. The catalyst of claim 17 wherein the inorganic binder is aluminum chlorohydrate.

18

19. The catalyst of claim 17 wherein the alumina is an acid or base peptized alumina.

20. The catalyst of claim 1 wherein the amount of inorganic binder ranges from about 10 to about 30 weight percent of the NO<sub>x</sub> reduction catalyst/additive composition.

21. The catalyst of claim 20 wherein the amount of inorganic binder present ranges from about 15 to about 25 weight percent of the NO<sub>x</sub> reduction catalyst/additive composition.

22. The catalyst of claim 1 wherein the NO<sub>x</sub> reduction zeolite component is selected from the group consisting of beta, MCM-49, mordenite, MCM-56, Zeolite-L, zeolite Rho, erionite, chabazite, clinoptilolite, MCM-22, Offretite, A, ZSM-12, ZSM-23, omega and mixtures thereof.

23. The catalyst of claim 1 wherein the NO<sub>x</sub> reduction zeolite component has a SiO<sub>2</sub> to Al<sub>2</sub>O<sub>3</sub> molar ratio of less than 500.

24. The catalyst of claim 1 wherein the particulate NO<sub>x</sub> catalyst/additive composition further comprises a zeolite other than the NO<sub>x</sub> reduction zeolite component.

25. The catalyst of claim 24 wherein the other zeolite is a zeolite selected from the group consisting of ferrierite, ZSM-5, ZSM-35 and mixtures thereof.

26. The catalyst of claim 24 wherein the other zeolite is present in an amount ranging from about 1 to about 80 weight percent of the NO<sub>x</sub> reduction catalyst/additive composition.

27. The catalyst of claim 26 wherein the other zeolite is present in an amount ranging from about 10 to about 70 weight percent of the NO<sub>x</sub> reduction catalyst/additive composition.

28. The catalyst of claim 1 wherein the composition further comprises a matrix material selected from the group consisting of alumina, silica, silica alumina, titania, zirconia, yttria, lanthana, ceria, neodymia, samaria, europia, gadolinia, praseodymia and mixtures thereof.

29. The catalyst of claim 28 wherein the matrix material is present in an amount less than 70 weight percent of the NO<sub>x</sub> reduction catalyst/additive composition.

30. The catalyst of claim 1 further comprising at least one additional NO<sub>x</sub> reduction composition.

31. The catalyst of claim 30 wherein the additional NO<sub>x</sub> reduction composition is a non-zeolitic composition.

32. The catalyst of claim 31 wherein the additional NO<sub>x</sub> reduction composition comprises (a) an acidic metal oxide containing substantially no zeolite; (b) a metal component, measured as the oxide, selected from the group consisting of an alkali metal, an alkaline earth metal and mixtures thereof; (c) an oxygen storage metal oxide component; and, (d) at least one noble metal component.

33. The catalyst of claim 30 wherein the additional NO<sub>x</sub> reduction composition comprises (a) an acidic metal oxide support; (b) an alkali metal, alkaline earth metal or mixtures thereof; (c) a transition metal oxide having oxygen storage capability; and, (d) a transition metal selected from Groups IB and IIB of the Periodic Table, and mixtures thereof.

34. The catalyst of claim 30 wherein the additional NO<sub>x</sub> reduction composition is a low NO<sub>x</sub> CO combustion promoter composition which comprises (a) an acidic oxide support; (b) an alkali metal, an alkaline earth metal or mixtures thereof; (c) a transition metal oxide having oxygen storage capability; and (d) palladium.

35. The catalyst of claim 30 wherein the additional NO<sub>x</sub> reduction composition comprises at least one metal-containing spinel which includes a first metal and a second metal having a valence higher than the valence of said first metal, at least one component of a third metal other than said first

19

and second metals and at least one component of a fourth metal other than said first, second and third metals, wherein said third metal is selected from the group consisting of Group IB metals, Group IIB metals, Group VIA metals, the rare-earth metals, the Platinum Group metals and mixtures thereof, and said fourth metal is selected from the group consisting of iron, nickel, titanium, chromium, manganese, cobalt, germanium, tin, bismuth, molybdenum, antimony, vanadium and mixtures thereof.

36. The catalyst of claim 35 wherein the metal containing spinel comprises magnesium as said first metal and aluminum as said second metal.

37. The catalyst of claim 35 wherein the third metal component in the metal containing spinel is selected from the group consisting of a Platinum Group metal, the rare-earth metals and mixtures thereof.

38. The catalyst of claim 35 wherein the third metal component is present in an amount in the range of about 0.001 to about 20 weight percent, calculated as elemental third metal.

39. The catalyst of claim 35 wherein said fourth metal component is present in an amount in the range of about 0.001 to about 10 weight percent, calculated as elemental fourth metal.

40. The catalyst of claim 30 wherein the additional  $\text{NO}_x$  reduction additive is a zinc based catalyst.

41. The catalyst of claim 30 wherein the additional  $\text{NO}_x$  reduction additive is an antimony based  $\text{NO}_x$  reduction additive.

42. The catalyst of claim 30 wherein the additional  $\text{NO}_x$  reduction additive is a perovskite-spinel  $\text{NO}_x$  reduction additive.

43. The catalyst of claim 30 wherein the additional  $\text{NO}_x$  reduction additive is a hydrotalcite containing composition.

44. The catalyst of claim 30 wherein the additional  $\text{NO}_x$  reduction composition comprises (i) an acidic metal oxide, (ii) cerium oxide, (iii) a lanthanide oxide other than ceria, and (iv) optionally, at least one oxide of a transition metal selected from Groups IB and IIB of the Periodic Table, and mixtures thereof.

45. The catalyst of claim 1 wherein the particulate  $\text{NO}_x$  reduction catalyst/additive composition has a mean particle size from about 50 to about 200  $\mu\text{m}$ .

46. The catalyst of claim 45 wherein the particulate  $\text{NO}_x$  reduction catalyst/additive composition has a mean particle size from about 55 to about 150  $\mu\text{m}$ .

47. The catalyst of claim 1 wherein the particulate  $\text{NO}_x$  reduction catalyst/additive composition has a Davison attrition index (DI) value of less than 50.

48. The catalyst of claim 47 wherein the particulate  $\text{NO}_x$  reduction catalyst/additive composition has a DI value of less than 20.

49. The catalyst of claim 48 wherein the particulate  $\text{NO}_x$  reduction catalyst/additive composition has a DI value of less than 15.

50. The catalyst of claim 3 wherein the ratio of  $\text{NO}_x$  reduction zeolite component to Y-type zeolite in the total catalyst inventory is less than 1.

51. A fluid cracking catalyst comprising (a) a cracking component suitable for catalyzing the cracking of hydrocarbons and (b) at least 0.1 weight percent of a  $\text{NO}_x$  reduction zeolite selected from the group consisting of ZSM-11, beta, MCM-49, mordenite, MCM-56, Zeolite-L, zeolite Rho, erionite, chabazite, clinoptilolite, MCM-22, MCM-35, MCM-61, Offretite, A, ZSM-12, ZSM-23, ZSM-18, ZSM-22, ZSM-57, ZSM-61, ZK-5, NaJ, Nu-87, Cit-1, SSZ-35, SSZ-48, SSZ-44, SSZ-23, Dachiardite, Merlinoite, Lovdarite,

20

Levyne, Laumontite, Epistilbite, Gmelonite, Gismondine, Cancrinite, Brewsterite, Stilbite, Paulingite, Goosecreekite, Natrolite, omega or mixtures thereof, wherein the  $\text{NO}_x$  reduction zeolite comprises at least one stabilizing metal selected from the group consisting of Groups 3B, 2A, 2B, 3A and the Lanthanide Series of the Periodic Table, and mixtures thereof.

52. The cracking catalyst of claim 51 wherein said catalyst comprises integral particles which contain both components (a) and (b).

53. The cracking catalyst of claim 51 wherein component (b) comprises from about 0.1 to about 60 wt % of the cracking catalyst.

54. The cracking catalyst of claim 53 wherein component (b) comprises from about 1 to about 40 wt % of the cracking catalyst.

55. The catalyst of claim 51 further comprising at least one additional  $\text{NO}_x$  reduction composition.

20 56. The catalyst of claim 55 wherein the additional  $\text{NO}_x$  reduction composition is a non-zeolitic composition.

57. The catalyst of claim 56 wherein the additional  $\text{NO}_x$  reduction composition comprises (a) an acidic metal oxide containing substantially no zeolite; (b) a metal component, measured as the oxide, selected from the group consisting of an alkali metal, an alkaline earth metal and mixtures thereof; (c) an oxygen storage metal oxide component; and (d) at least one noble metal component.

30 58. The catalyst of claim 55 wherein the additional  $\text{NO}_x$  reduction composition comprises (a) an acidic metal oxide support; (b) an alkali metal, alkaline earth metal or mixtures thereof (c) a transition metal oxide having oxygen storage capability; and, (d) a transition metal selected from Groups IB and IIB of the Periodic Table, and mixtures thereof.

59. The catalyst of claim 55 wherein the additional  $\text{NO}_x$  reduction composition is a low  $\text{NO}_x$  CO combustion promoter composition which comprises (a) an acidic oxide support; (b) an alkali metal, an alkaline earth metal or mixtures thereof (c) a transition metal oxide having oxygen storage capability; and (d) palladium.

60 60. The catalyst of claim 55 wherein the additional  $\text{NO}_x$  reduction composition comprises at least one metal-containing spinel which includes a first metal and a second metal having a valence higher than the valence of said first metal, at least one component of a third metal other than said first and second metals and at least one component of a fourth metal other than said first, second and third metals, wherein said third metal is selected from the group consisting of Group IB metals, Group IIB metals, Group VIA metals, the rare-earth metals, the Platinum Group metals and mixtures thereof, and said fourth metal is selected from the group consisting of iron, nickel, titanium, chromium, manganese, cobalt, germanium, tin, bismuth, molybdenum, antimony, vanadium and mixtures thereof.

61. The catalyst of claim 60 wherein the metal containing spinel comprises magnesium as said first metal and aluminum as said second metal.

62. The catalyst of claim 60 wherein the third metal component in the metal containing spinel is selected from the group consisting of a Platinum Group metal, the rare-earth metals and mixtures thereof.

63. The catalyst of claim 60 wherein the third metal component is present in an amount in the range of about 0.001 to about 20 weight percent, calculated as elemental third metal.

**21**

**64.** The catalyst of claim **60** wherein said fourth metal component is present in an amount in the range of about 0.001 to about 10 weight percent, calculated as elemental fourth metal.

**65.** The catalyst of claim **55** wherein the additional  $\text{NO}_x$  reduction additive is a zinc based catalyst.

**66.** The catalyst of claim **55** wherein the additional  $\text{NO}_x$  reduction additive is an antimony based  $\text{NO}_x$  reduction additive.

**67.** The catalyst of claim **55** wherein the additional  $\text{NO}_x$  reduction additive is a pervoskite-spinel  $\text{NO}_x$  reduction additive.

**68.** The catalyst of claim **55** wherein the additional  $\text{NO}_x$  reduction additive is a hydrotalcite containing composition.

**69.** The catalyst of claim **55** wherein the additional  $\text{NO}_x$  reduction composition comprises (i) an acidic metal oxide, (ii) cerium oxide, (iii) a lanthanide oxide other than ceria, and (iv) optionally, at least one oxide of a transition metal selected from Groups IB and IIB of the Periodic Table, and mixtures thereof.

**70.** The catalyst of claim **51** wherein component (a) comprises a Y-type zeolite and component (b) is present in an amount sufficient to provide a ratio of  $\text{NO}_x$  reduction zeolite to Y-type zeolite of less than 2 in the total catalyst.

**71.** The catalyst of claim **70** wherein component (b) is present in an amount sufficient to provide a ratio of  $\text{NO}_x$  reduction zeolite to Y-type zeolite of less than 1 in the total catalyst.

**72.** The catalyst of claim **51** wherein the stabilizing metal is selected from the group consisting of lanthanum, aluminum, magnesium and zinc, and mixtures thereof.

**22**

**73.** The catalyst of claim **51** wherein the stabilizing metal is incorporated into the pores of component (b).

**74.** The catalyst of claim **51** wherein the  $\text{NO}_x$  reduction zeolite is selected from the group consisting of beta, MCM-49, mordenite, MCM-56, Zeolite-L, zeolite Rho, erionite, chabazite, clinoptilolite, MCM-22, Offretite, A, ZSM-12, ZSM-23, omega and mixtures thereof.

**75.** The catalyst of claim **51** wherein the  $\text{NO}_x$  reduction zeolite has a  $\text{SiO}_2$  to  $\text{Al}_2\text{O}_3$  molar ratio of less than 500.

**76.** The catalyst of claim **51** further comprising a zeolite other than the  $\text{NO}_x$  reduction zeolite.

**77.** The catalyst of claim **76** wherein the other zeolite is selected from the group consisting of ferrierite, ZSM-5, ZSM-35 and mixtures thereof.

**78.** The catalyst of claim **76** or **77** wherein the other zeolite is present in an amount ranging from about 1 to about 80 weight percent of the composition.

**79.** The catalyst of claim **78** wherein the other zeolite is present in an amount ranging from about 10 to about 70 weight percent of the composition.

**80.** The catalyst of claim **51** wherein the  $\text{NO}_x$  reduction zeolite is exchanged with a cation selected from the group consisting of hydrogen, ammonium, alkali metal and combinations thereof.

\* \* \* \* \*

UNITED STATES PATENT AND TRADEMARK OFFICE  
**CERTIFICATE OF CORRECTION**

PATENT NO. : 7,304,011 B2  
APPLICATION NO. : 10/824913  
DATED : December 4, 2007  
INVENTOR(S) : George Yaluris, Michael Scott Ziebarth and Xinjin Zhao

Page 1 of 1

It is certified that error appears in the above-identified patent and that said Letters Patent is hereby corrected as shown below:

In Claim 1, Col. 17, line 8, delete “alumina phosphate” and insert --aluminum phosphate--.

Signed and Sealed this  
Seventeenth Day of May, 2011



David J. Kappos  
*Director of the United States Patent and Trademark Office*